

## UNITED STATES PATENT OFFICE.

LINN BRADLEY, OF MONTCLAIR, NEW JERSEY, AND EDWARD P. MCKEEFE, OF PLATTSBURG, NEW YORK.

## PRODUCTION OF PULP.

No Drawing. Original application filed March 28, 1921, Serial No. 456,187. Divided and this application filed April 10, 1924. Serial No. 705,711.

To all whom it may concern:

Be it known that we, LINN BRADLEY and EDWARD P. MCKEEFE, both citizens of the United States, residing at Montclair, county 5 of Essex, State of New Jersey, and Plattsburg, county of Clinton, State of New York, respectively, have invented certain new and useful Improvements in the Production of Pulp; and we do hereby declare the following 10 to be a full, clear, and exact description of the invention, such as will enable others skilled in the art to which it appertains, to make and use the same.

This invention relates to improvements in processes of cooking wood chips and similar material for the production of wood cellulose products or pulp.

The present invention includes a new method of cooking or digesting wood chips 20 in which the cooking liquor is an alkaline liquor containing a thiosulfate of an alkali, or both a sulfite and a thiosulfate of an alkali. This method is distinguished by the fact that caustic soda is present in sufficient 25 amounts to give an alkaline cooking liquor of appropriate strength, while sodium thiosulfate, or both sodium sulfite and sodium thiosulfate, is or are also present in substantial 30 amounts. The composite cooking liquor, containing caustic soda and sodium thiosulfate, or containing caustic soda together with sodium sulfite and sodium thiosulfate, can vary somewhat in its composition and in the proportions of caustic soda 35 and of sodium thiosulfate, or of sodium thiosulfate and sodium sulfite. Ordinarily a preponderating proportion of caustic soda will be used, for example, so that from 50 to 90% of the total sodium of the cooking 40 liquor will be present as caustic soda and the remainder mainly as sodium thiosulfate, or as sodium sulfite and sodium thiosulfate. A cooking liquor may thus be used containing at least 40 gr. of sodium per liter, of 45 which at least 40% is present as sodium hydroxide and at least 5% as sodium thiosulfate, or as sodium sulfite and sodium thiosulfate, with the particular amounts of caustic soda and sodium thiosulfate, or of sodium thiosulfate and sodium sulfite, varying somewhat above these percentages. The 50 amount of cooking liquor may be about 700 to 1100 gallons for a cord of wood (meas-

ured before chipping), the liquor containing the higher percentages of caustic soda being used in smaller amount, and those containing the smaller percentages of caustic soda being used in larger amount. By the use of such an alkaline cooking liquor containing thiosulfate, or thiosulfate and sulfite, it is possible to produce satisfactory pulp or cellulose material from forest products and other cellulose-bearing materials which, due to their inherent composition and properties, have been unsuited to the 60 production of high grade cellulose material by the processes heretofore commonly practiced. Materials such as woods and other forest material of inferior value (for treatment according to common methods) as well 65 as materials such as bagasse, reeds, grasses, bamboo, cornstalks, straw, etc., can advantageously be subjected to digestion with such alkaline thiosulfate, or sulfite and thiosulfate, cooking liquor and high grade pulp or 70 cellulose material produced therefrom. This method, therefore, increases the available supply of raw materials for the production of high grade pulp or cellulose 75 products. 80

In carrying out the digestion with such an alkaline thiosulfate liquor, or with such an alkaline sulfite and thiosulfate liquor, the time of treatment and the temperature, pressure, etc., can be varied depending upon 85 the particular wood or other material undergoing digestion; but the process can be carried out under similar conditions of temperature and pressure to those commonly 90 used in the soda process, e. g., by heating the digester by direct steam at a pressure which may vary for about 90 to 140 lbs., and with circulation of the liquor within the digester by the steam during the digestion. The digestion will, however, be modified by the action of the composite cooking liquor so that 95 less injury to the cellulose material will take place and so that a superior pulp or cellulose material will be produced.

According to the present invention, accordingly, the alkaline cooking liquor may be composed of caustic soda and sodium thiosulfate, or it may be composed of three ingredients, namely, caustic soda, sodium sulfite and sodium thiosulfate. The liquor 100 may also contain other compounds than 105

those mentioned, such, for example, as sodium sulfate, sodium carbonate, or sodium sulfide.

Our investigations have shown that if some untreated black liquor is mixed with new cooking liquor containing caustic soda, a portion of the caustic soda is used up in the formation of other sodium compounds by reaction either directly or indirectly between the caustic soda and soluble organic compounds, so that the total content of caustic soda is not available for cooking the wood chips in the same way that it would be if no such soluble organic constituents were present. Sodium sulfite and sodium thiosulfate exert a retarding influence upon the reaction between the caustic soda and the soluble organic compounds, and likewise upon the cellulose, so that the caustic soda can act more effectively, and so that the destructive action for the same total amount of caustic soda is minimized.

The present application is a division of our prior application, Serial No. 456187, filed March 28, 1921.

We claim:

1. The improvement in the production of pulp, which comprises subjecting the wood chips in the digester to the action of a cooking liquor containing caustic soda and sodium thiosulfate, the caustic soda being present in preponderating amount.

2. In the preparation of chemical pulp, the use of a cooking liquor comprising sodium hydroxide and sodium thiosulfate, the sodium hydroxide being used materially in excess of the amount required to decompose silicates and aluminates in the material treated.

40 3. In the preparation of chemical pulp,

the use of a cooking liquor comprising a hydroxide and a thiosulfate, the hydroxide being used materially in excess of the amount required to decompose silicates and aluminates in the material treated. 45

4. In the preparation of chemical pulp, the use of a cooking liquor comprising a hydroxide and a thiosulfate, the hydroxide being present in preponderating amount.

5. In the preparation of chemical pulp, the use of a cooking liquor comprising sodium hydroxide and sodium thiosulfate, the sodium hydroxide being present in preponderating amount. 50

6. The improvement in the production of pulp, which comprises subjecting wood chips in a digester to the action of a cooking liquor containing caustic soda and sodium thiosulfate, the caustic soda constituting from 50 to 90 per cent of the total sodium 60 of the cooking liquor.

7. The improvement in the production of pulp, which comprises subjecting wood chips to digestion with a cooking liquor containing caustic soda and sodium thiosulfate, 65 the cooking liquor containing at least 40 grams of sodium per liter, of which at least 40 per cent is present as sodium hydroxide and at least 5 per cent as sodium thiosulfate.

8. The method of minimizing the destructive action of caustic soda upon the soluble organic compounds of wood in the cooking of wood chips, which comprises cooking the chips with a caustic soda cooking liquor containing sodium thiosulfate in amount less 75 than that of the caustic soda.

In testimony whereof we hereunto affix our signatures.

LINN BRADLEY.  
EDWARD P. MCKEEFE.